

April 25, 1972

YORIKATSU IRISAKA ET AL

3,658,713

ALKALI METAL GENERATING AGENTS

Filed Nov. 10, 1969

9 Sheets-Sheet 1



April 25, 1972

YORIKATSU IRISAKA ET AL

3,658,713

ALKALI METAL GENERATING AGENTS

Filed Nov. 10, 1969

9 Sheets-Sheet 2



April 25, 1972

YORIKATSU IRISAKA ET AL

3,658,713

ALKALI METAL GENERATING AGENTS

Filed Nov. 10, 1969

9 Sheets-Sheet 3

FIG. 2A



FIG. 2C



April 25, 1972

YORIKATSU IRISAKA ET AL

3,658,713

ALKALI METAL GENERATING AGENTS

Filed Nov. 10, 1969

9 Sheets-Sheet 4

FIG. 2B



REPRODUCIBILITY (  $\frac{\text{NO. OF GOOD PRODUCTS}}{\text{NO. OF TESTS}} \times 100$  ) %

April 25, 1972

YORIKATSU IRISAKA ET AL

3,658,713

ALKALI METAL GENERATING AGENTS

Filed Nov. 10, 1969

9 Sheets-Sheet 5



April 25, 1972

YORIKATSU IRISAKA ET AL

3,658,713

ALKALI METAL GENERATING AGENTS

Filed Nov. 10, 1969

9 Sheets-Sheet 6



April 25, 1972

YORIKATSU IRISAKA ET AL

3,658,713

ALKALI METAL GENERATING AGENTS

Filed Nov. 10, 1969

9 Sheets-Sheet 7



April 25, 1972

YORIKATSU IRISAKA ET AL

3,658,713

ALKALI METAL GENERATING AGENTS

Filed Nov. 10, 1969

9 Sheets-Sheet 8

FIG. 7A



FIG. 7B



April 25, 1972

YORIKATSU IRISAKA ET AL

3,658,713

ALKALI METAL GENERATING AGENTS

Filed Nov. 10, 1969

9 Sheets-Sheet 9

FIG. 8



FIG. 9



3,658,713

**ALKALI METAL GENERATING AGENTS**  
 Yorikatsu Irisaka, Yokohama-shi, and Haruo Takashio,  
 Tokyo, Japan, assignors to Tokyo Shibaura Electric  
 Co., Ltd., Kawasaki-shi, Japan  
 Filed Nov. 10, 1969, Ser. No. 875,064  
 Claims priority, application Japan, Nov. 12, 1968,  
 43/82,303  
 Int. Cl. H01v 39/22; C22b 27/00  
 U.S. CL. 252—181.4

16 Claims

**ABSTRACT OF THE DISCLOSURE**

Alkali metal generating agents generally used in forming a photosensitive layer, characterized in that they consist of a mixture of alkali metal salts and niobium. The mixture is put in a vessel made of electric conductive material to form a generator. When the generator is heated both materials react with each other to allow the alkali metal to come out of the vessel and form the aforementioned layer.

The present invention relates to alkali metal generating agents and more particularly to said agents put in a vessel made of electric conductive material so as jointly to form an alkali metal generator.

Alkali metal generating agents heretofore used in forming the photoconductive target or surface of a special tube such as an image pickup tube or photoelectric tube consist of a mixture of a single or plurality of alkali metal salts and a single or plurality of reducing agents. The mixture is received in a vessel made of electric conductive material and perforated with a plurality of small bores to form a generator.

There are selectively used various kinds of alkali metal salts according to the type of a photosensitive layer employed. The known types of said salts include chromates, bichromates, tungstates and molybdenates of sodium, potassium, cesium, lithium and rubidium. And the known types of reducing agents are mainly silicon, zirconium, aluminum and boron.

Such prior art alkali metal generator is previously disposed in the prescribed part of a tube at which there is to be formed a photosensitive layer. Where it is required to form said layer, the metal vessel is heated by introduction of current or high frequency induction for reaction between the alkali metal salts and reducing agents so as to release alkali metals. The alkali metal thus released is deposited on the surface of a photoelectric substrate, for example, an antimony film previously conditioned for this purpose by maintaining a part of the tube at a suitable level of temperature, thereby forming a photosensitive layer or surface through a further prescribed process.

The aforementioned metal vessel is fabricated by rolling a thin electric conductive sheet in the transverse direction, to form a hollow cylindrical body, spot welding the superposed edge portions at a plurality of points arranged in the longitudinal direction at a prescribed interval and finally closing up an opening at both ends of the hollow cylindrical body by pressure. The aforesaid spot welding is intended to allow the released alkali metal to be drawn out of the vessel through the gaps formed between the welds.

With the prior art alkali metal generator having the aforesaid arrangement, it is required to heat the generator up to the temperature at which there occurs the exothermic reaction of the above-mentioned mixture in order to release a relatively large amount of alkali metal from a given amount of alkali metal salt used. However, heating of the generator to such high level of temperature leads to a rapid occurrence of reaction, thus present-

ing difficulties in controlling the amount of alkali metal to be released.

To prevent such rapid occurrence of reaction, the prior art adds tungsten as a buffer agent to mixtures of alkali salts and reducing agents. However, even addition of said tungsten failed reliably to control the aforementioned rapid reaction. Accordingly, a photosensitive layer obtained by the prior art could not display a desired degree of photosensitivity, nor was fully satisfactory in other respects.

It is accordingly the object of the present invention to provide an alkali metal generating agent capable of easily controlling the velocity of exothermal reaction which raised a problem with the prior art, by adding niobium as a reducing agent to the alkali metal salt and forming a photosensitive layer or surface having excellent properties and also an alkali metal generator prepared by putting said generating agent in a vessel made of electric conductive metal.

This invention can be more fully understood from the following detailed description when taken in connection with reference to the accompanying drawings, in which:

FIGS. 1A and 1B are diagrams comparing the amount of alkali metal released from the prior art alkali metal generating agents corresponding to the associated temperature with that of a similar agent according to an embodiment of the present invention;

FIGS. 2A to 2C illustrate the effect of a kind of alkali metal generating agent according to the invention and the relationship of the yield of alkali metal in forming a photosensitive film versus the ratio in which there are blended the components of said agent;

FIGS. 3A and 3B are similar diagrams to FIG. 1A comparing the alkali metal generating property associated with Example D of the invention with those of the prior art alkali metal generating agents;

FIG. 4 is a diagram indicating the relationship between the blending ratio of an alkali metal salt and niobium constituting the generating agent used in said Example D and the temperature required for said generation;

FIGS. 5A and 5B are similar diagrams to FIGS. 3A and 3B associated with the alkali metal generating agent of Example E;

FIG. 6 is a similar diagram to FIG. 4 associated with Example E;

FIGS. 7A and 7B are similar diagrams to FIGS. 5A and 5B associated with the alkali metal generating agent of Example F;

FIG. 8 is a similar diagram to FIG. 6 associated with Example F; and

FIG. 9 is a perspective view, with part broken away, of an example of an alkali metal generator filled with the generating agent of the invention.

For better understanding of the present invention, there will now be described the prior art reducing agents. Reaction of the prior art reducing agents such as silicon, aluminium and zirconium with alkali metal salts is of exothermic type. Among said reducing agents, silicon causes a tremendous evolution of heat. And all these reactions, except between cesium chromate and zirconium, take place very rapidly. Even addition, as heretofore attempted, of powdered tungsten as a buffer agent for suppressing the above-mentioned rapidity of reaction fails to control reaction velocity with respect to other alkali metal generating agents than a mixture of zirconium and potassium chromate. Although a mixture of zirconium and alkali metal salts allows its reaction velocity to be appreciably controlled as described above, there will most likely take place an explosion during reaction, so that said mixture is barred from use. Where the aforementioned both components are slowly mixed dry in the forming of relatively coarse powders, said explosion may be avoided.

TABLE 1

| Mixture                               | Photo-sensitivity, $\mu\text{A}/\text{cm}^2$ | Generated state | Generated state affected by varying pre-heating conditions | Gas evolution before generation of alkali metal | Control of generated state | Getter action of reductant | True density (g./cm. <sup>3</sup> ) | Bulk density (g./cm. <sup>3</sup> ) | Addition of buffer agent | Possibility of explosion | Yield of alkali metal (percent) |
|---------------------------------------|----------------------------------------------|-----------------|------------------------------------------------------------|-------------------------------------------------|----------------------------|----------------------------|-------------------------------------|-------------------------------------|--------------------------|--------------------------|---------------------------------|
| Nb+Cs <sub>2</sub> CrO <sub>4</sub>   | 2:1                                          | 100             | Very stable...                                             | ca. 780                                         | Never...                   | Little affected...         | Very small...                       | Great...                            | 6.42                     | 2.4                      | None...                         |
| Si+Cs <sub>2</sub> CrO <sub>4</sub>   | 2:1                                          | 50              | Unstable...                                                | ca. 900                                         | Sometimes...               | Noticeably affected...     | Prominent...                        | Small...                            | 2.745                    | 0.9                      | Necessary...                    |
| Zn+Cs <sub>2</sub> CrO <sub>4</sub>   | 2:1                                          | 60              | Stable...                                                  | ca. 900                                         | Quite rare...              | Affected...                | Fairly noticeable...                | Great...                            | 5.32                     | 1.8                      | Preferred...                    |
| Nb+K <sub>2</sub> CrO <sub>4</sub>    | 2:1                                          | Very stable...  | ca. 800                                                    | Never...                                        | Little affected...         | Very small...              | do...                               | do...                               | 6.07                     | 2.1                      | Unnecessary...                  |
| Si+K <sub>2</sub> CrO <sub>4</sub>    | 2:1                                          | Unstable...     | ca. 900                                                    | Sometimes...                                    | Noticeably affected...     | Prominent...               | Easy...                             | do...                               | 2.45                     | 0.9                      | Necessary...                    |
| Zn+K <sub>2</sub> CrO <sub>4</sub>    | 2:1                                          | Stable...       | ca. 900                                                    | Quite rare...                                   | Affected...                | Fairly noticeable...       | Fairly easy...                      | Small...                            | 4.44                     | 1.2                      | Preferred...                    |
| Si+K <sub>2</sub> CrO <sub>4</sub> +W | 2:1                                          | do...           | ca. 900                                                    | Sometimes...                                    | do...                      | Prominent...               | do...                               | do...                               | 11.95                    | 3.1                      | Already contained...            |
| Zn+K <sub>2</sub> CrO <sub>4</sub> +W | 2:1                                          | do...           | ca. 900                                                    | Quite rare...                                   | do...                      | do...                      | do...                               | do...                               | 8.75                     | 2.1                      | Present...                      |

to a certain extent. However, such process does not afford uniform mixing, nor does use of coarse powders assist in the reduction of the surface area of zirconium taking part in reaction. Accordingly, if it is desired to generate a

- 5 prescribed amount of alkali metal, it is necessary to use a large amount of the aforesaid mixture. On the other hand, wet mixing of zirconium and alkali metal salts can indeed prevent the occurrence of an explosion. But the alkali metal salt is dissolved in water to become useless.
- 10 Even where alcohol is used in place of water, minute amounts of water contained in the alcohol denature the alkali metal salt and the segregation of said salt in the subsequent drying process reduces the uniformity of said mixture, thus failing to form a satisfactory photosensitive layer.

15 The prior art alkali metal generator is generally pre-heated to minimize the evolution, during reaction, of unnecessary gases from the alkali metal salts, reducing agents and metal vessel used. However, said preheating has the drawback that there are evolved during reaction different amounts of such unnecessary gases from a mixture of an alkali metal salt and silicon or zirconium, depending on the condition in which said preheating is conducted.

20 Heretofore, there has been further proposed a different type of an alkali metal generator capable of generating appreciable amounts of alkali metal at relatively low temperature, wherein there are added powders of tungsten and boron to a mixture of alkali metal salts and reducing agents. Even this generator, however, presents difficulties in controlling reaction velocity.

25 The different properties of the prior art alkali metal generating mixture and the mixture of the present invention which typically consists of alkali metal salts and niobium are presented in FIGS. 1A and 1B and Table 1 below. The ordinate of the figures represents the amount of alkali metal generated (the ordinate of FIG. 1A denotes cesium and that of FIG. 1B potassium) and the abscissa indicates heating temperature ( $^{\circ}\text{C}$ ).

30 Table 1 does not include an alkali metal generating agent containing aluminium as a reducing agent. Such generating agent resembles those containing silicon and zirconium in respect of property, but evolves tremendous amounts of gas during reaction, failing to provide a good photosensitive layer. On the other, use of scale-like pieces of aluminium can indeed suppress gas evolution to a certain extent, but there is required an extra process of working aluminium itself into such scale-like pieces.

35 There will now be described the present invention in greater detail. It is preferred that powders of alkali metal salts and those of niobium filled into a vessel made of electric conductive metal from which alkali metal is released be mixed in the ratio by weight ranging from 1:0.1 to 8. The reason is that in the ratio of 1:less than 0.1, the content of niobium is too small to display its expected effect, whereas in the ratio of 1:more than 8, there likely takes place a rapid exothermic reaction. Further speaking of the effect caused by the content of niobium.

40 (A) Where the alkali metal salt consists of potassium chromate ( $\text{K}_2\text{CrO}_4$ ), it is advisable to mix it with niobium in the ratio by weight of about 1:0.1 to 8 (or in the mol ratio of about 1:0.23 to 18.4), preferably in the ratio by weight of about 1:0.3 to 4 (or in the mol ratio of about 1:0.69 to 9.2). The mol number of alkali metal represents that of salts thereof. Hereinafter, the mol number of alkali salts is expressed by drawing a bar above symbols representing alkali elements, as  $\overline{\text{Na}}$ ,  $\overline{\text{K}}$ ,  $\overline{\text{Cs}}$ . The mol number of for example,  $\text{Na}_2\text{CrO}_4$  or  $\text{K}_2\text{WO}_4$ , is denoted as  $\overline{\text{Na}}$  or  $\overline{\text{K}}$ . This is derived from the fact that where there was manufactured a photoelectric tube using an alkali metal generating agent whose components were mixed in the forming ratio, the yield of alkali metal accounted for about 90 to 100 percent and in the case of the latter mixing ratio approximately 100 percent.

45 (B) Where the alkali metal salt consists of cesium chromate ( $\text{Cs}_2\text{CrO}_4$ ), it is desired that said salt be mixed

with niobium in the ratio by weight of about 1:0.3 to 10 (or in the mol ratio of about 1:1.21 to 40.49), preferably in the ratio by weight of about 1:0.5 to 3 (or in the mol ratio of about 1:2.02 to 12.12).

(C) In case sodium chromate is used as an alkali metal salt, the advisable ratio by weight of said salt to niobium is about 1:0.1 to 10 (or about 1:0.19 to .19 in the mol ratio).

There was formed a photosensitive layer from the aforementioned alkali metal salts, i.e., potassium chromate, cesium chromate and sodium chromate mixed with niobium in varying proportions, the yield of alkali metal being presented in FIGS. 2A, 2B and 2C respectively. Throughout these figures, the ordinate represents the percentage yield of alkali metal or reproducibility (number of good products/number of tests  $\times 100$ ) and the abscissa denotes the ratio by weight of niobium to the aforementioned alkali metal salts.

As described above and indicated in Table 1, the alkali metal generator of the present invention allows alkali metal to be released at a temperature about 100° C. lower than required for the prior art, reduces the evolution of unnecessary gas, eliminates the necessity of using any special buffer agent and easily controls reaction velocity because reaction does not occur rapidly. Moreover, the generated state of alkali metal does not widely vary with changes in the conditions in which preheating is conducted prior to application of heat for reaction, and on this account, too, reaction velocity can be easily controlled. The fact that the photosensitive layer prepared from the alkali metal generating agent of the present invention is elevated about 70 percent in photosensitivity over the prior art layer evidently proves that said agent is prominently excellent with respect to the aforementioned requirements.

The alkali metal generator of the present invention further offers the undermentioned favourable effect. The alkali metal generating agent of the invention generally has a greater bulk density than the prior art agent (for example, where the alkali metal salt consists of cesium chromate and there is added niobium thereto as claimed in the present invention, the entire mass has a bulk density of 2.4 g./cm.<sup>3</sup>, whereas the prior art agent containing silicon amounts to 0.9 g./cm.<sup>3</sup> in bulk density and that containing zirconium to 1.8 g./cm.<sup>3</sup>. This means that the alkali metal generating agent of the present invention has a bulk density about 2.5 times that of the prior art silicon-bearing agent and about 1.3 times that of the prior art zirconium-containing agent). Accordingly, the alkali metal generating agent of the present invention can be reduced in bulk, permitting a vessel of electric conductive metal to be made compact. Also the fact that relatively small amounts of said alkali metal generating agent are used and reaction can proceed at a relatively low temperature naturally decreases the evolution of unnecessary gas during the exothermic reaction. Furthermore, the present alkali metal generating agent enables alkali metal to be released in a prominently elevated yield. Though the reason is not fully understood, it is assumed that the intermediate product probably formed by reaction between niobium and the alkali metal generating agent is less liable to obstruct the release of alkali metal than the intermediate product supposed to occur during the reaction of the prior art alkali metal generating mixture.

For illustration of other combinations of alkali metal potassium tungstate ( $K_2WO_4$ ) and niobium mixed in different ratios as given below.

| Sample: | Ratio by weight of Nb to $K_2WO_4$ | Mol ratio of K to Nb |
|---------|------------------------------------|----------------------|
| a.....  | 0.33:1                             | 2:1.17               |
| b.....  | 1:1                                | 2:3.5                |
| c.....  | 3:1                                | 2:10.5               |
| d.....  | 9:1                                | 2:31.5               |

In any of the above ratios, the present invention displayed its claimed effect of easily controlling reaction velocity and realizing the initial generation of alkali metal at a temperature of about 700° C.

5 A further combination of alkali metal salts and niobium wherein there were mixed sodium molybdenate



and niobium in the mol ratio  $\bar{Na}/Nb$  of 2 to 0.07 exhibited the same effect as described above.

10 In addition to the aforementioned kinds of alkali metal salts involved in the alkali metal generating agents according to the present invention, there may be used others alone or in combination. Said other salts can still display 15 the same effect as mentioned above. There will now be described the concrete examples where there were used said other salts in combination.

(D) There is used a mixture of sodium and potassium salts as a source of alkali metal. The respective salts

20 are mixed in such a manner that the mol ratio of the total amount of sodium and potassium salts constituting said source to the niobium is about 1:0.2 to 50

$$[(Na+K/Nb=0.02 \text{ to } 5)]$$

25 It is also experimentally disclosed that when the mol ratio of sodium and potassium is  $\bar{Na}/\bar{K}=0.1$  to 10 the resultant photosensitive layer has good photosensitivity.

(E) There are mixed salts of cesium and potassium to form a source of alkali metal in such a manner that 30 the mol ratio of the total amount of cesium and potassium salts constituting said source to the niobium is about 1:0.2 to 100  $[(\bar{Cs}+\bar{K})/Nb=0.01 \text{ to } 5)]$ . In this case, the cesium and potassium mixed in the mol ratio of 1:0.5 to 10 ( $\bar{Cs}/\bar{K}=0.1$  to 20) affords good results.

35 (F) There are mixed salts of cesium and sodium as a source of alkali metal in such a manner that the mol ratio of the total amount of cesium and sodium salts constituting said source to the niobium is about 1:0.125 to 100  $[(\bar{Cs}+\bar{Na})/Nb=0.01 \text{ to } 8)]$ . In this case, too, the mixing of cesium and sodium in the mol ratio of 1:0.03 to 10 ( $\bar{Cs}/\bar{Na}=0.1$  to 30) displays a good effect.

40 The aforementioned metal salts used as a source of alkali metal include, for example, chromates, bichromates, tungstates and molybdenates.

45 The present invention will be more fully understood from the examples which follow:

#### EXAMPLES A, B AND C

50 There were mixed powders of cesium chromate, potassium chromate and sodium chromate respectively with powders of niobium in the mol ratio of 1:2 to form an alkali metal generating agent. The properties of these mixtures are presented in FIGS. 1A and 1B, FIGS. 2A and 2B, and Tables 1 and 2.

#### EXAMPLE D

55 There were mixed powders of sodium chromate and potassium chromate in such a manner that the mol ratio of sodium to potassium was  $\bar{Na}/\bar{K}=1$ . Further, the mixture and powders of niobium were mixed in the mol ratio of  $(\bar{Na}+K/\bar{Nb}=0.2$  to form an alkali metal generating agent.

60 For comparison with the aforementioned generating agent of the present invention, there was prepared a reference alkali metal generating agent by adding silicon and zirconium respectively in amounts equal to the aforementioned mol ratio of niobium to the above-described mixed powders of sodium chromate and potassium chromate. The alkali metal generating agents of the present invention and prior art were respectively charged into a perforated vessel made of electric conductive metal to form a photosensitive layer or surface. With respect to the above-mentioned three kinds of mixtures including the alkali metal generating agent of the present invention 70 containing niobium and the reference generating agents 75 containing niobium and the reference generating agents

containing silicon and zirconium respectively, there was investigated the generated state of sodium and potassium corresponding to the temperature at which said three generating agents were heated, the results being given in FIGS. 3A and 3B. There are further presented in Table 2 below comparative data on said three mixtures, the condition of a layer during formation and its properties after formation.

## EXAMPLE E

There were mixed powders of cesium chromate and potassium chromate in such a manner that the cesium and potassium contained therein had a mol ratio of  $\overline{\text{Cs}}/\overline{\text{K}}=4$ . To said mixture were further added powders of niobium in the mol ratio of  $(\overline{\text{Cs}}+\overline{\text{K}})/\text{Nb}=0.1$  to form an alkali metal generating agent according to the present invention.

TABLE 2

| Alkali metal generating agent                                       | $\text{Nb}+\text{Na}_2\text{CrO}_4+\text{K}_2\text{CrO}_4$                             | $\text{Si}+\text{Na}_2\text{CrO}_4$<br>$+ \text{K}_2\text{CrO}_4$                          | $\text{Zr}+\text{Na}_2\text{CrO}_4$<br>$+ \text{K}_2\text{CrO}_4$                          |
|---------------------------------------------------------------------|----------------------------------------------------------------------------------------|--------------------------------------------------------------------------------------------|--------------------------------------------------------------------------------------------|
| Mol ratio of components                                             | $\begin{cases} \text{Na}/\text{K}=1 \\ (\text{Na}+\text{K})/\text{Nb}=0.2 \end{cases}$ | $\begin{cases} \text{Na}/\text{K}=1 \\ (\text{Na}+\text{K})/\text{Zr} \\ =0.2 \end{cases}$ | $\begin{cases} \text{Na}/\text{K}=1 \\ (\text{Na}+\text{K})/\text{Zr} \\ =0.2 \end{cases}$ |
| Photosensitivity $\mu\text{A}/\text{lm.}$ ( $n$ : number of sample) | 100 ( $n=5$ )                                                                          | 70 ( $n=5$ )                                                                               | 80 ( $n=5$ )                                                                               |
| Generated state                                                     | Very stable                                                                            | Unstable                                                                                   | Stable                                                                                     |
| Temperature of generation, $^{\circ}\text{C.}$                      | About 780                                                                              | About 900                                                                                  | About 900                                                                                  |
| Puncture or breakage by melting                                     | Never                                                                                  | Sometimes                                                                                  | Quite rare                                                                                 |
| Generated state affected by varying preheating conditions           | Little affected                                                                        | Noticeably affected                                                                        | Affected                                                                                   |
| Gas evolution before generation of alkali metal                     | Very small                                                                             | Prominent                                                                                  | Fairly noticeable                                                                          |
| Control of generated state                                          | Easy                                                                                   | Difficult                                                                                  | Fairly easy                                                                                |
| Getter action of reductant                                          | Great                                                                                  | Small                                                                                      | Great                                                                                      |
| Bulk density                                                        | 2.4                                                                                    | 0.9                                                                                        | 1.8                                                                                        |
| Addition of buffer agent                                            | Unnecessary                                                                            | Necessary                                                                                  | Preferred                                                                                  |
| Possibility of explosion                                            | None                                                                                   | None                                                                                       | Present                                                                                    |
| Yield of alkali metal                                               | High                                                                                   | Low                                                                                        | Medium                                                                                     |

When there was added to the alkali metal generating agent of the present invention used in this example about 10 percent by weight of tungsten or aluminium oxide on the basis of the total amount of said agent, there was better controlled the generation of alkali metal or reaction velocity.

There was further investigated the temperature of generation using the same materials (mixture of sodium and potassium) as used in this Example D with the mol ratio of niobium to said mixture varied. The results are presented in FIG. 4 wherein the ordinate denotes the temperature  $^{\circ}\text{C.}$  required for the generation of alkali metal and the abscissa represents the mol ratio of niobium to said mixture.

40 Next for comparison, there were prepared reference alkali metal generating agents corresponding to the prior art agent, using silicon and zirconium respectively as a reducing agent in place of niobium with all the components mixed in the same mol ratio as is used in the present invention. There was investigated the amount of cesium and 45 potassium generated from said three kinds of generating agents containing niobium, silicon and zirconium respectively, the data on cesium and potassium being presented in FIGS. 5A and 5B respectively. There were also tested the properties of a photosensitive layer prepared from these three kinds of generating agents, the results being given in Table 3 below.

TABLE 3

| Alkali metal generating agent                                       | $\text{Nb}+\text{Cs}_2\text{CrO}_4+\text{K}_2\text{CrO}_4$                                                   | $\text{Si}+\text{Cs}_2\text{CrO}_4$<br>$+ \text{K}_2\text{CrO}_4$                          | $\text{Zr}+\text{Cs}_2\text{CrO}_4$<br>$+ \text{K}_2\text{CrO}_4$                          |
|---------------------------------------------------------------------|--------------------------------------------------------------------------------------------------------------|--------------------------------------------------------------------------------------------|--------------------------------------------------------------------------------------------|
| Mol ratio of components                                             | $\begin{cases} \overline{\text{Cs}}/\overline{\text{K}}=4 \\ (\text{Cs}+\text{K})/\text{Nb}=0.1 \end{cases}$ | $\begin{cases} \text{Cs}/\text{K}=4 \\ (\text{Cs}+\text{K})/\text{Si}= \\ 0.1 \end{cases}$ | $\begin{cases} \text{Cs}/\text{K}=4 \\ (\text{Cs}+\text{K})/\text{Zr}= \\ 0.1 \end{cases}$ |
| Photosensitivity $\mu\text{A}/\text{lm.}$ ( $n$ : number of sample) | 100 ( $n=5$ )                                                                                                | 70 ( $n=5$ )                                                                               | 80 ( $n=5$ )                                                                               |
| Generated state                                                     | Very stable                                                                                                  | Unstable                                                                                   | Stable                                                                                     |
| Temperature of generation, $^{\circ}\text{C.}$                      | About 780                                                                                                    | About 900                                                                                  | About 900                                                                                  |
| Puncture or breakage by melting                                     | Never                                                                                                        | Sometimes                                                                                  | Quite rare                                                                                 |
| Generated state affected by varying preheating conditions           | Little affected                                                                                              | Noticeably affected                                                                        | Affected                                                                                   |
| Gas evolution before generation of alkali metal                     | Very small                                                                                                   | Prominent                                                                                  | Fairly noticeable                                                                          |
| Control of generated state                                          | Easy                                                                                                         | Difficult                                                                                  | Fairly easy                                                                                |
| Getter action of reductant                                          | Great                                                                                                        | Small                                                                                      | Great                                                                                      |
| Bulk density                                                        | 2.4                                                                                                          | 0.9                                                                                        | 1.8                                                                                        |
| Addition of buffer agent                                            | Unnecessary                                                                                                  | Necessary                                                                                  | Preferred                                                                                  |
| Possibility of explosion                                            | None                                                                                                         | None                                                                                       | Present                                                                                    |
| Yield of alkali metal                                               | High                                                                                                         | Low                                                                                        | Medium                                                                                     |

There is further indicated in FIG. 6 the temperature required for generation of cesium and potassium with respect to the mixing ratio of Nb to  $\bar{Cs} + \bar{K}$ . In this figure, the ordinate denotes the temperature required for generation of said alkali metals and the abscissa represents the mol ratio of Nb to  $\bar{Cs} + \bar{K}$ .

## EXAMPLE F

There were mixed powders of cesium chromate ( $Cs_2CrO_4$ ) and sodium chromate ( $Na_2CrO_4$ ) in the mol ratio of  $\bar{Cs}/\bar{Na}=3$ . To this mixture was added niobium in the mol ratio of  $(\bar{Cs} + \bar{Na})/Nb=1$  to form an alkali metal generating agent according to the present invention. There were also prepared prior art generating agents containing silicon and zirconium respectively in the same manner as

5

15

alkali metal salt to the aforesaid alkali metal salts used in combination. There will now be described a concrete example of this case.

There were mixed powders of cesium chromate ( $Cs_2CrO_4$ ), potassium chromate ( $K_2CrO_4$ ) and sodium chromate ( $Na_2CrO_4$ ) in such a manner that  $\bar{Cs}$ ,  $\bar{K}$  and  $\bar{Na}$  are contained in the mol ratio of 1:1:1. To said mixture was further added niobium in the mol ratio of

$$(\bar{Cs} + \bar{K} + \bar{Na})/Nb=0.2$$

to form an alkali metal generating agent according to the present invention. There were comparatively studied the properties of said agent consisting of only one alkali metal and niobium, namely,  $Nb + K_2WO_4$  or  $Nb + NaMoO_4$ , the results being presented in Table 5 below.

TABLE 5

| Alkali metal generating agent                            | $Nb + K_2WO_4$  | $Nb + NaMoO_4$  | $Nb + Cs_2CrO_4 + K_2CrO_4 + Na_2CrO_4$                             |
|----------------------------------------------------------|-----------------|-----------------|---------------------------------------------------------------------|
| Mol ratio of components                                  | $K/Nb=0.2$      | $Na/Nb=0.2$     | $\{Cs: K: Na=1:1:1$<br>$(\bar{Cs} + \bar{K} + \bar{Na})/Nb=0.2-9.0$ |
| Generated state                                          | Very stable     | Stable          | Stable                                                              |
| Temperature of generation, °C                            | 700             | 700             | 780                                                                 |
| Puncture or breakage by melting                          | Never           | Never           | Never                                                               |
| Generated state affected by varying preheating condition | Little affected | Little affected | Slightly affected                                                   |
| Gas evolution before generation of alkali metal          | Small           | Small           | Small                                                               |
| Control of generated state                               | Very easy       | Easy            | Easy                                                                |
| Addition of buffer agent                                 | Unnecessary     | Unnecessary     | Unnecessary                                                         |
| Possibility of explosion                                 | None            | None            | None                                                                |
| Yield of alkali metal                                    | High            | Medium          | High                                                                |
| Bulk density                                             | 2.4             | 2.4             | 2.4                                                                 |

in Example E. Data of comparative study on the alkali metal generating agents of the present invention and prior art are given in FIGS. 7A and 7B and Table 4 below formed in the same arrangement as used in FIGS. 5A and 5B and Table 3 respectively. The temperature of generation associated with FIGS. 7A and 7B is presented in FIG. 8 formed in the same arrangement as in FIG. 6.

45

As mentioned above, the present invention is characterized in that there is mixed niobium with alkali metal salts. However, there may be further added to said mixture a material, for example, zirconium used as a reducing agent and/or gettering material in the prior art. There are presented in Table 6 below the properties of a zirconium containing alkali metal generating agent in com-

TABLE 4

| Alkali metal generating agent                             | $Nb + Cs_2CrO_4 + Na_2CrO_4$                            | $Si + Cs_2CrO_4 + Na_2CrO_4$                          | $Zr + Cs_2CrO_4 + Na_2CrO_4$                          |
|-----------------------------------------------------------|---------------------------------------------------------|-------------------------------------------------------|-------------------------------------------------------|
| Mol ratio of components                                   | $\{\bar{Cs}/\bar{Na}=3$<br>$(\bar{Cs} + \bar{Na})/Nb=1$ | $\bar{Cs}/\bar{Na}=3$<br>$(\bar{Cs} + \bar{Na})/Si=1$ | $\bar{Cs}/\bar{Na}=3$<br>$(\bar{Cs} + \bar{Na})/Zr=1$ |
| Photosensitivity $\mu A/lm.$ ( $n$ : number of sample)    | 100 ( $n=6$ )                                           | 70 ( $n=5$ )                                          | 80 ( $n=5$ )                                          |
| Generated state                                           | Very stable                                             | Unstable                                              | Stable                                                |
| Temperature of generation, °C                             | About 780                                               | About 900                                             | About 900                                             |
| Puncture or breakage by melting                           | Never                                                   | Sometimes                                             | Quite rare                                            |
| Generated state affected by varying preheating conditions | Little affected                                         | Noticeably affected                                   | Affected                                              |
| Gas evolution before generation of alkali metal           | Very small                                              | Prominent                                             | Fairly noticeable                                     |
| Control of generated state                                | Easy                                                    | Difficult                                             | Fairly easy                                           |
| Getter action of reductant                                | Great                                                   | Small                                                 | Great                                                 |
| Bulk density                                              | 2.4                                                     | 0.9                                                   | 1.8                                                   |
| Addition of buffer agent                                  | Unnecessary                                             | Necessary                                             | Preferred                                             |
| Possibility of explosion                                  | None                                                    | None                                                  | Present                                               |
| Yield of alkali metal                                     | High                                                    | Low                                                   | Medium                                                |

To the present invention may be applicable a different alkali metal generating agent prepared by adding another

parison with those of other agents of the present invention.

75

TABLE 6

|                                                                | I                                      | II                                                                      | III                                      | IV                                          | V                                   | VI                                                                   | VII                                |
|----------------------------------------------------------------|----------------------------------------|-------------------------------------------------------------------------|------------------------------------------|---------------------------------------------|-------------------------------------|----------------------------------------------------------------------|------------------------------------|
| Alkali metal generating agent.....                             | Nb+Si+Cs <sub>2</sub> CrO <sub>4</sub> | Nb+Si+K <sub>2</sub> CrO <sub>4</sub> +Na <sub>2</sub> CrO <sub>4</sub> | Nb+Si+Zr+K <sub>2</sub> CrO <sub>4</sub> | Nb+Si+Zr+W+Cs <sub>2</sub> CrO <sub>4</sub> | Si+Cs <sub>2</sub> CrO <sub>4</sub> | Si+K <sub>2</sub> CrO <sub>4</sub> +Na <sub>2</sub> CrO <sub>4</sub> | Zr+K <sub>2</sub> CrO <sub>4</sub> |
| Mol ratio of components.....                                   | Cs/(Nb+Si)=0.2                         | (K+Na)/(Nb+Si)=0.2                                                      | K/(Nb+Zr)=0.2                            | Cs/(Nb+Si+Zr+W)=0.2                         | Cs/Si=0.2                           | Cs/Si=0.2                                                            | K/Zr=0.2                           |
| Photosensitivity, $\mu$ A/lm.....                              | 100                                    | 100                                                                     | 100                                      | 100                                         | 50                                  | 70                                                                   | 70                                 |
| Generated state.....                                           | Very stable.....                       | Very stable.....                                                        | Very stable.....                         | Very stable.....                            | Unstable.....                       | Unstable.....                                                        | Stable.....                        |
| Temperature of generation, °C.....                             | About 780.....                         | About 780.....                                                          | About 800.....                           | About 800.....                              | About 900.....                      | About 900.....                                                       | About 900.....                     |
| Puncture or breakage by melting.....                           | Quite rare.....                        | Never.....                                                              | Quite rare.....                          | Never.....                                  | Sometimes.....                      | Sometimes.....                                                       | Quite rare.....                    |
| Generated state affected by varying preheating conditions..... | Little affected.....                   | Little affected.....                                                    | Little affected.....                     | Little affected.....                        | Noticeably affected.....            | Noticeably affected.....                                             | Affected.....                      |
| Gas evolution before generation of alkali metal.....           | Very small.....                        | Very small.....                                                         | Very small.....                          | Very small.....                             | Great.....                          | Great.....                                                           | Fairly noticeable.....             |
| Control of generated state.....                                | Easy.....                              | Easy.....                                                               | Easy.....                                | Easy.....                                   | Difficult.....                      | Difficult.....                                                       | Fairly easy.....                   |
| Gether action of reductant.....                                | Great.....                             | Great.....                                                              | Great.....                               | Great.....                                  | Small.....                          | Small.....                                                           | Great.....                         |
| Bulk density.....                                              | 2.4.....                               | 2.0.....                                                                | 2.0.....                                 | 2.0.....                                    | 3.2.....                            | 0.9.....                                                             | 1.2.....                           |
| Addition of buffer agent.....                                  | Unnecessary.....                       | Unnecessary.....                                                        | Unnecessary.....                         | Unnecessary.....                            | Necessary.....                      | Necessary.....                                                       | Preferred.....                     |
| Possibility of explosion.....                                  | None.....                              | None.....                                                               | None.....                                | None.....                                   | None.....                           | None.....                                                            | Present.....                       |
| Yield of alkali metal.....                                     | About 80%.....                         | About 80%.....                                                          | About 80%.....                           | About 75%.....                              | About 75%.....                      | Low.....                                                             | About 50%.....                     |

There will now be described by reference to FIG. 9 the case where there is actually prepared a photosensitive layer for a special image pickup tube. Numeral 10 is a vessel made of electric conductive metal. The vessel is prepared by rolling, for example, a thin metal sheet once crosswise into a cylindrical body, and spot welding the longitudinal edge portions at a prescribed interval to form a slight gap 12 between the welds 11. The vessel 10 is filled with an alkali metal generating agent according to the present invention. After the agent is charged, the wall of each end of the vessel is pressed airtight.

There will now be described the case where there was formed the antimony-cesium photosensitive layer of a head-on type photoelectric tube, using an alkali metal generator two alkali metal generators filled with a generating agent consisting of a mixture of powdered cesium chromate and powdered niobium and a generating agent consisting of a mixture of powdered potassium chromate and powdered niobium respectively. Each mixture weighed 70 mg. and the mol ratio of the alkali metal salt to niobium was chosen to be 1:2. To the curved lateral inner surface of a glass bulb having a face plate at the front part were fitted each alkali metal generator and a known antimony generator by so bending them as to correspond to the curvature of said lateral inner surface of the glass bulb. To both ends of each of these fitted generators are connected lead wires drawn to the outside. The preparatory step for forming the aforesaid layer ended by disposing secondary electron multiplying electrodes known to this particular field and an anode at prescribed locations respectively. First, the glass bulb was fully evacuated and then there was introduced current through said antimony generator containing an antimony generating agent. Said agent was heated to a temperature of 520 to 570° C. to release antimony so as to deposit a thin film thereof on the inner surface of said face plate to a prescribed thickness. Thereafter, the two alkali metal generators of the present invention were preheated 5 minutes at a temperature of 600° C. by introducing current therethrough. The generators were further heated to 900° C. to release potassium and cesium. Thus, there was deposited a thin cesium-potassium film on said antimony substrate to form a photosensitive layer.

The photosensitive layer prepared as described above had a photosensitivity of 100  $\mu$ A/lm., showing that it had excellent properties.

There will now be described the formation of a multialkali photosensitive layer used in an X-ray fluorescent multiplying tube. There were prepared three mixtures comprising powders of cesium chromate, sodium chromate and potassium chromate each blended with powders of niobium in the mol ratio of 1:2 to form alkali metal generating agents. The mixtures containing cesium and sodium each weighing 250 mg. and the mixture containing potassium weighing 200 mg. were separately placed in the aforementioned metal vessels to provide alkali metal generators. Each of these generators was put in a known bulb having a fluorescent face formed at one end and a plate of insulating material disposed opposite to said fluorescent face at a close interval. The generators were preheated 5 to 10 minutes at a temperature of 350° C. Then they were heated to 900° C. to release each alkali metal so as to form a multialkali photosensitive layer on said insulation plate. The resultant photosensitive layers had an excellent photosensitivity of 100  $\mu$ A/lm. like that of the preceding case.

What we claim is:

1. An alkali metal generating composition comprising a mixture of an alkali metal salt and niobium in a ratio by weight of salt to niobium of from about 1:0.1 to about 10.
2. A composition according to claim 1 wherein the alkali metal salt is selected from the group consisting of potassium tungstate, potassium chromate, cesium chromate, sodium chromate and sodium molybdate.

## 13

3. A composition according to claim 2 wherein the alkali metal salt is potassium chromate, and wherein the weight ratio of said chromate to niobium is 1:0.1 to 8.

4. A composition according to claim 2 wherein the alkali metal salt is cesium chromate, and wherein the weight ratio of said chromate to niobium is 1:0.3 to 10.

5. A composition according to claim 2 wherein the alkali metal salt is sodium chromate, and wherein the weight ratio of said chromate to niobium is 1:0.1 to 10.

6. A composition according to claim 1 wherein said alkali metal salt is cesium chromate and which further contains silicon and wherein the mol ratio of Cs/Nb+Si is about 0.2.

7. A composition according to claim 1 wherein said alkali metal salt is potassium chromate and which further contains zirconium and wherein the mol ratio of K/Nb+Zr is about 0.2.

8. A composition according to claim 1 wherein said alkali metal salt is cesium chromate and which further contains silicon, zirconium and tungsten and wherein the mol ratio of Cs/Nb+Si+Zr+W is about 0.2.

9. A composition according to claim 1 wherein said alkali metal salt is a mixture of cesium chromate, potassium chromate and sodium chromate and, wherein the molar ratio of Cs:K:Na is about 1:1:1.

10. A composition according to claim 1 wherein the alkali metal salt is selected from the group consisting of a first mixture of sodium salts and potassium salts, a second mixture of cesium salts and potassium salts and a third mixture of cesium salts and sodium salts.

## 14

11. A composition according to claim 10 wherein the mol ratio of the total amount of sodium and potassium salts of said first mixture to niobium is from 1:0.2 to .50.

12. A composition according to claim 11 wherein the mol ratio of sodium salt to potassium salt of said first mixture is from 0.1 to 10.

13. A composition according to claim 10 wherein the mol ratio of the total amount of cesium salt and potassium salt of said second mixture to niobium is from 1:0.2 to 100.

14. A composition according to claim 13 wherein the mol ratio of cesium salt to potassium salt of said second mixture is from 0.1 to 20.

15. A composition according to claim 10 wherein the mol ratio of the total amount of cesium salt and sodium salt of said third mixture to niobium is from 1:0.125 to 10.

16. A composition according to claim 10 wherein the mol ratio of cesium salt to sodium salt of said third mixture is from 0.1 to 30.

## References Cited

## UNITED STATES PATENTS

|           |         |             |       |             |
|-----------|---------|-------------|-------|-------------|
| 2,154,131 | 4/1939  | Lelever     | ----- | 252—181.4 X |
| 2,173,258 | 9/1939  | Lelever     | ----- | 252—181.4   |
| 1,835,118 | 12/1931 | Marden      | ----- | 252—181.4 X |
| 3,096,211 | 7/1963  | Davis       | ----- | 252—181.4 X |
| 3,468,807 | 9/1969  | Spangenberg | ----- | 252—181.4   |

TOBIAS E. LEVOW, Primary Examiner

30 J. COOPER, Assistant Examiner

UNITED STATES PATENT OFFICE  
CERTIFICATE OF CORRECTION

Patent No. 3,658,713 Dated April 25, 1972

Inventor(s) YORIKATSU IRISAKA et al

It is certified that error appears in the above-identified patent and that said Letters Patent are hereby corrected as shown below:

Column 5, line 63 - after "metal" insert "salts and niobium, there were prepared four samples from".

Signed and sealed this 5th day of December 1972.

(SEAL)  
Attest:

EDWARD M. FLETCHER, JR.  
Attesting Officer

ROBERT GOTTSCHALK  
Commissioner of Patents